

E. A. ASHCROFT,  
PROCESS AND APPARATUS FOR THE ELECTROLYTIC DECOMPOSITION OF ANHYDROUS  
MAGNESIUM CHLORID AND THE PRODUCTION OF MAGNESIUM OR  
ALLOYS THEREOF AND CHLORIN.  
APPLICATION FILED AUG. 12, 1919.

1,359,653.

Patented Nov. 23, 1920.

3 SHEETS—SHEET 1.



Fig. 1.

*Inventor:*  
Edgar A. Ashcroft  
*by his Attorney:*  
Howson and Howson

E. A. ASHCROFT.  
PROCESS AND APPARATUS FOR THE ELECTROLYTIC DECOMPOSITION OF ANHYDROUS  
MAGNESIUM CHLORID AND THE PRODUCTION OF MAGNESIUM OR  
ALLOYS THEREOF AND CHLORIN.  
APPLICATION FILED AUG 12, 1919.

1,359,653.

Patented Nov. 23, 1920.

3 SHEETS—SHEET 2.



Fig. 2.

Inventor.  
Edgar A. Ashcroft.  
by his Attorney,  
Howson and Howson

E. A. ASHCROFT.  
PROCESS AND APPARATUS FOR THE ELECTROLYTIC DECOMPOSITION OF ANHYDROUS  
MAGNESIUM CHLORID AND THE PRODUCTION OF MAGNESIUM OR  
ALLOYS THEREOF AND CHLORIN.  
APPLICATION FILED AUG. 12, 1919.

1,359,653.

Patented Nov. 23, 1920.

3 SHEETS—SHEET 3.



Inventor  
Edgar A. Ashcroft.  
by his Attorneys,  
Hawson and Hawson

# UNITED STATES PATENT OFFICE.

EDGAR ARTHUR ASHCROFT, OF LONDON, ENGLAND.

## PROCESS AND APPARATUS FOR THE ELECTROLYTIC DECOMPOSITION OF ANHYDROUS MAGNESIUM CHLORID AND THE PRODUCTION OF MAGNESIUM OR ALLOYS THEREOF AND CHLORIN.

1,359,653.

Specification of Letters Patent. Patented Nov. 23, 1920.

Application filed August 12, 1919. Serial No. 317,083.

To all whom it may concern:

Be it known that I, EDGAR ARTHUR ASHCROFT, a subject of the King of Great Britain, residing at 65 London Wall, in the city of London, England, have invented new and useful improved processes and apparatus for the electrolytic decomposition of anhydrous magnesium chlorid and the production of magnesium or alloys thereof and chlorin, of which the following is a specification.

The principal object of my invention is to provide an efficient process and apparatus whereby an electrolyte consisting of anhydrous magnesium chlorid alone, (or practically alone), can be resolved into its elements (magnesium metal and chlorin gas) and the magnesium metal can be obtained pure.

It is well known that the electrolytic production of the metal magnesium from magnesium chlorid alone has never yet been possible in practice, and the general practice is to use, in the electrolytic cell, a double salt of magnesium and potassium, or the like, for instance carnallite, to which is often added calcium fluorid, the extraneous salts constituting fluxes. It is furthermore (and in consequence of the presence of such fluxing salts) the general practice in existing processes to periodically dismantle the cell and gather the magnesium by allowing it to set in the electrolyte and afterward to break the solidified electrolyte and separate the magnesium therefrom and purify it by refusion.

Such operations are exceedingly expensive and troublesome and moreover the presence of other metal salt in the electrolyte, according to the well known laws of mass reaction and electrolytic dissociation, unavoidably causes impurity to be deposited into the magnesium while impurity is also gathered unavoidably by the process of frequently dismantling the cell.

It has also been suggested to use such composite electrolytes and to receive the metal into some more electro-positive metal afterward recovering it therefrom by secondary electrolysis, the electro-positive metals proposed for this purpose being copper alumini-

um and tin. I have found, by experiment, that by none of these combinations can the pure metal be produced. The process according to my present invention can be carried out as follows.

I employ a twin cell electrolytic apparatus each cell being constructed preferably of cast steel and the respective cells being preferably alike in construction and design, but reversed in position relatively to each other. At the bottom of the said cell is a body of molten lead (preferably alloyed with about 5 to 10 per cent. of magnesium) the level being maintained constant by a weir extending across the cell and communicating with an outlet pocket, the other end of the cell communicating with an outlet pocket. The part of the cell which is exposed to the fused electrolyte is lined with refractory material such for instance as fire-clay, or magnesia bricks, or tiles. The primary cell is fitted with a cover from which depend anodes, preferably of graphite, in electrical connection with the cover, but insulated from the cell. The primary electrolyte is superimposed on the magnesium lead alloy. The said electrolyte consists of fused anhydrous magnesium chlorid alone, or practically alone as far as the introduction of objectionable impurities into the product is concerned. The electrolyte is consumed by the passage of the current and fresh quantities of crystalline anhydrous magnesium chlorid are added to maintain the electrolyte at the same level while the magnesium produced is received into the molten lead alloy.

In the secondary cell the reverse process takes place. An unconsumed and unchangeable body of electrolyte consisting also of magnesium chlorid alone, or practically alone as aforesaid, is superimposed upon the alloy at the bottom of the cell. The cover of this cell is fitted with depending cathodes, consisting of iron, or steel, rods which dip into the secondary electrolyte and receive the deposit of magnesium, which floats in the said electrolyte. This cover is preferably fitted with separately removable sectional covers closing openings in the main cover so that access can be had to the cell

for the removal of magnesium from time to time without removing the main cover, or otherwise disturbing the action of the process. The secondary electrolyte is continuously renewed by solution of fresh magnesium from the alloy.

During the passage of the current at suitable intervals the interchange of the alloy between the secondary cell and the primary cell is brought about by any convenient means; for instance, by simultaneous ladling, or otherwise transferring, the molten alloy from pocket to pocket, at the respective ends of the adjacent twin cells.

15 The process according to my invention is thus a continuous one and may be carried on with a minimum of labor and with great durability of apparatus. Anhydrous magnesium chlorid alone, or practically alone, 20 is the only material employed and this is employed quantitatively in relation to the magnesium produced while the chlorin gas is also evolved quantitatively. In the secondary cell the product of magnesium is 25 also obtained quantitatively, and in a very high degree of purity.

To show the enormously improved working of the process according to my invention as against those hitherto employed I give 30 the following data obtained from actual operation, but it is to be understood that I do not limit myself to the details given.

Current efficiency 90 to 95 per cent. volts at the terminals of the primary cell, 4 to 6 35 volts according to the current density employed; volts at the secondary cell, 1 to 2.5 volts according to current density employed. The current density employed may conveniently be such that the surplus energy 40 evolved is sufficient to maintain the contents of the vat in fusion. I have found the most suitable as follows:—For an apparatus taking 5000 amperes I employ say twenty anodes, preferably of graphite, each about 3 45 inches in diameter and immersed about three inches in the electrolyte and one inch distant from the surface of the cathodic metal alloy while in the secondary cell I preferably employ four movable covers each of which may 50 be fitted with say 70 depending cathodes of iron, or steel, each being about say three-eighths of an inch in diameter and immersed half an inch in the electrolyte and three quarters of an inch distant from the surface 55 of the anodic metal alloy. Under these conditions I obtain a terminal voltage of 6 volts for the primary cell and 2 volts for the secondary cell. I maintain the temperature of both cells at about 750° centigrade which I 60 have found gives the best results.

The anhydrous magnesium chlorid for the purposes of my invention may be obtained from ordinary crystalline hydrated magnesium chlorid of commerce by subjecting it 65 to any suitable drying, or dehydrating, proc-

ess, I prefer however to employ that described in the specification of my application No. 317,082 for Letters Patent of even date herewith. The said anhydrous magnesium chlorid is fused and used alone (or practically alone) as the electrolyte.

I will now describe how my process may be performed and the apparatus be constructed with reference to the accompanying drawings but I do not limit myself to the precise details.

Figure 1 is a longitudinal section, Fig. 2 a plan, and Fig. 3 a transverse section of the apparatus, which comprises primary and secondary cells (preferably made of cast 80 steel) which, through their bodies are in electrical connection with each other as shown at  $\alpha$ . The said cells may be of identical form, or construction, except in respect to the covers and electrodes as hereinafter described. Each of the said cells has a main part, or cell-proper, (marked respectively 1 and 2) in communication, by passages 4 and 5 at the bottom, with opposite pockets, 6 and 7, one pocket being for introducing the alloy 85 of magnesium and lead and the other being for withdrawing the alloy, the passage to the pocket 7 from the cell-proper being preceded, in the cell-proper, by a weir 8 extending across from side to side of the cell and rising to a height the same as that to which the alloy is required to rise, the walls of the cell-proper rising to a greater height to hold the fused electrolyte and provide space for gaseous chlorin and to support the anodes 90 in the primary cell and the cathodes 10, in the secondary cell, by suitable insulated covers 11 and 12 which close the respective cells. The portion of the cell-proper 1 and 2 above the level of the top of the weir 8 105 should be lined with fire-clay 13, or other suitable refractory, or protective, material and the undersides of the covers be similarly protected. The cells are arranged as a pair (or in two, or more, pairs) side by side 110 and close together in such relative positions that the alloy which is withdrawn from the primary cell 1 can be conveniently transferred to the secondary cell 2 and vice versa. The primary cell 1, has anodes 9, preferably 115 of graphite, the alloy of lead and magnesium constituting the cathodes in this cell, while the secondary cell 2 has cathodes 10 of iron, or steel, the lead and magnesium alloy constituting the anode in this cell. In this double 120 cell arrangement the electric current passes through the two cells 1 and 2 in series, the anodes 9, in the first cell 1, forming the positive pole and the iron, or steel, cathodes 10, in the secondary cell 2, forming the negative 125 pole of the pair, while the molten alloy body forms a secondary, or intermediate, electrode. Any required number of such pairs can be connected in series if desired.

I prefer to mount the anodes 9 in open- 130

ings in the cover 11 of the primary cell 1 and attach them by cementing or the like, electrical connection being secured by providing a number of suitable conductors, 14, to the 5 cover (which is in the electric circuit) of the cell which securing can be readily done by introducing the respective ends of the said conductors 14 into holes, in the cover, at one end and corresponding holes in the anodes 10 9 at the other end, molten lead being run in the holes to secure good electrical connection.

I prefer to carry the cathodes 10 in sets attached to any suitable number (say four) 15 of supplementary covers 15, which are applied to openings in the main cover 12 which is in the electric circuit, each supplementary cover 15 being connected to the main cover 12 by a flexible conductor 16, so that any 20 supplementary cover 15, with the set of cathodes 10 which it carries, can be instantly removed by means of the handle 17 and be replaced without disturbing the rest of the apparatus.

25 In operating these cells a portion of the alloy, as it increases in volume by the addition of magnesium, passes over the weir 8 and into the pocket beyond, from which it is withdrawn and can be introduced into the 30 secondary cell 2 through the adjacent pocket thereof. The alloy is passed, or caused to pass, periodically from cell to cell as hereinafter described. The electrolytic action of the current in the secondary cell causes 35 the magnesium metal to collect at the iron, or steel, cathodes, the said metal floating on the electrolyte in molten condition. This magnesium metal, being uncontaminated by impurities, (which is an important advan- 40 tage as against other processes for the production of magnesium), does not require re-fusion but may be ladled from the cell and, for instance cast directly into any desired molds, or used directly in the extrusion process. I have found that no lead is 45 deposited with the magnesium metal and that the pure, or practically pure, chlorid electrolyte prepared as aforesaid has no solvent action either on the magnesium de- 50 posited, or on the lead of the alloy so that a perfect, or almost perfect, current efficiency is obtained. The conductivity is also extremely good.

In working the said cells the alloy should 55 be allowed to remain tranquil, for a time, during the passage of the current, say for about six hours for each gathering of the metal, the voltage of the cell terminals remaining constant during this run because 60 the slight shrinkage of the alloy in the secondary cell is found to increase the resistance in the same proportion as the accumulation of the magnesium around the cathodes reduces the resistance. The magnesium

metal floats in large masses in the fused elec- 65 trolyte. When the magnesium metal has sufficiently accumulated in the secondary cell the small covers and the cathodes thereof are successively removed, and the magnesium can then be readily ladled from the 70 electrolyte and the cover and cathodes be afterward replaced without the passage of the current having been interrupted, the whole operation occupying only a few minutes. From time to time, (preferably im- 75 mediately after the gathering of the magnesium as hereinbefore explained), the alloy is passed briskly through the cells, from cell to cell, which can be done, for example, by ladling the alloy from the pocket of the 80 primary cell and pouring it back into the pocket of the connected secondary cell, the pockets being conveniently arranged in reverse juxtaposition, as aforesaid, for the purpose. Or any convenient mechanical de- 85 vice, or arrangement of communicating pas- sages, may be employed to effect the trans- ference of the alloy. The openings 18 and 19 in the covers of the respective cells are for the introduction of the electrolyte. 90

What I claim is—

1. For use in the electrolytic decomposi- 95 tion of anhydrous magnesium chlorid and the production of magnesium metal and chlorin, a double electrolytic apparatus com- 100 prising two cells electrically connected in series through their body-parts and each having pockets, passages at the bottoms of the cells establishing communication be- 105 tween said pockets, and a weir across each cell at a height approximately the same as that to which the alloy-body in each cell has to rise, the walls of each cell-proper rising to a greater height than the said alloy-body, and being adapted to contain the fused elec- 110 trolyte and afford space for the gaseous products escaping during the decomposition of the electrolyte, covers for both cells, a high carbon anode supported in the cover in the primary cell, and an iron cathode sup- 115 ported in the cover in the secondary cell.

2. For use in the electrolytic decomposi- 120 tion of anhydrous magnesium chlorid and the production of magnesium metal and chlorin, a double electrolytic apparatus of 125 the construction specified in claim 1, a cover for the secondary cell having openings therein, supplementary covers applied to said openings, cathodes carried in sets at- tached to said supplementary covers, each of said supplementary covers being con- 130 nected to the said main cover by a flexible conductor so that any one of the said sup- plementary covers, with the set of cathodes which it carries, can be removed and re- placed without disturbing the rest of the ap- 135 paratus or interrupting the electric current.

3. For use in the electrolytic decomposi-

tion of anhydrous magnesium chlorid and the production of magnesium metal and chlorin in the double cell arrangement specified in claim 1, an electrolyte in both primary and secondary cells consisting substantially solely of pure magnesium chlorid.

In testimony whereof I have signed my

name to this specification in the presence of two subscribing witnesses.

EDGAR ARTHUR ASHCROFT.

Witnesses:

G. F. LYONS,  
L. WALTER.